

April 23, 1968

J. A. SPICER

3,378,900

METHOD OF BULKING YARNS

Filed Feb. 23, 1966



FIG. 1



FIG. 2

Inventor

J. A. SPICER

Davis, Hoxie, <sup>By</sup> & Hough  
Happgood Attorneys

1

3,378,900

**METHOD OF BULKING YARNS**

Jack Albert Spicer, Coventry, England, assignor to  
Courtaulds Limited, London, England, a British  
company

Filed Feb. 23, 1966, Ser. No. 535,283  
2 Claims. (Cl. 28—72)

**ABSTRACT OF THE DISCLOSURE**

A yarn bulking process comprising passing a plurality of low-twist, heat-settable, continuous filament yarns between nip rollers and through a stuffing box in which the yarns are allowed a degree of lateral movement, heating the yarns at some stage in their passage through the stuffing box, cooling the yarns to set the crimp imposed on them in the stuffing box, stretching the yarns to separate the filaments in the yarns, and then relaxing the yarns, whereupon the filaments tend to revert to their crimped shapes and engagement of adjacent filaments with each other produces a bulking effect on the yarns.

This invention relates to the production of bulked yarns.

It is already known to produce crimped yarns and fibres by forcing them by means of positively fed rollers into a confined space, generally described as a stuffing box, through which the yarns or fibres are forced against the friction of the walls of the box to emerge at the far end. In the box, the individual fibres or yarns assume a crimped configuration and the extent to which this is retained in the yarn which emerges can be enhanced by the application of heat to the yarn or fibre in the box.

According to the present invention a yarn bulking process comprises passing a plurality of low-twist, heat-settable, continuous filament yarns, parallel to each other and in a single layer, between a pair of nip rollers into and through a stuffing box comprising a channel of width such that the yarns are allowed a degree of lateral movement, the open side of the channel being closed by a pressure plate, heating the yarns in or before entering the stuffing box, cooling the yarns to set the crimp imposed on them in the stuffing box, stretching the yarns to at least 90 percent of their uncrimped lengths, thereby separating the filaments in the yarns, and then relaxing the yarns, whereupon the filaments tend to revert to the crimped shapes imparted to them in the stuffing box, and engagement of adjacent filaments with each other produces a bulking effect on the yarns.

By "low twist" yarns we mean yarns with a twist of up to about 5 turns per inch. In practice the process is best applied to yarns having only a spinning twist, that is about  $\frac{1}{3}$ — $\frac{1}{2}$  turn per inch.

The term "heat-settable" as applied to yarns which may be bulked by the process, means that each yarn should contain a sufficient proportion of thermoplastic filaments for the yarns to be set in the shape imparted to them during the process. Preferably the yarns consist wholly of thermoplastic filaments.

Heating the yarns may be accomplished in or before they enter the stuffing box. With heavy denier yarns it may even be necessary to heat the yarns both before and within the stuffing box. When the stuffing box is itself heated, this is generally accomplished electrically. Additional heating may be provided by admitting steam to the stuffing box through apertures provided in the channel and/or the pressure plate for this purpose.

By virtue of the lateral spacing of the yarns in the

2

stuffing box, they are permitted to crimp laterally as well as against the restraining force of the pressure plate, and this lateral crimping causes filaments of adjacent yarns to interfere with each other, although the yarns themselves are prevented from overlapping and maintained in a single layer by the pressure plate. This interference causes the adjacent yarns to cling together, and the yarns are delivered from the stuffing box in the form of a flat ribbon. On stretching the ribbon, the filaments are straightened out so that the interfering filaments, and consequently the individual yarns, are separated, and the yarns can then be relaxed and wound separately into packages in their bulked state, or fed directly to subsequent processing equipment.

The stretching operation may be accomplished immediately after the yarns have cooled or, if desired, the stretching operation may be delayed. Thus, in practice, it may be convenient to pack the ribbon of crimped yarns delivered from the stuffing box directly into a box or bale and then, when it is desired to bulk the yarn, the individual yarns can be separated by drawing the ribbon from the box or bale through a tensioning zone where the filaments are substantially straightened and through a relaxation zone.

By a "plurality" of yarns is meant at least two but the number may rise to the limit of the number of yarns which can be controlled in the stuffing box. There must not, of course, be so many yarns in relation to the width of the stuffing box that the yarns are not allowed a degree of lateral movement. More than one layer of yarns, each layer comprising a plurality of yarns in side-by-side relation may be passed into the stuffing box if desired. By the suitable choice of the numbers of yarns in each layer and by the superimposition of yarns in upper layers upon yarns in lower layers, a "doubling" effect is obtainable by keeping pairs or groups of superimposed yarns close together during the relaxation, so that filaments of the adjacent yarns again tend to interfere to keep the yarns together, and the joined yarns may in fact be used without further treatment. Using this doubling effect it is possible to obtain heavy denier yarns containing a large number of low denier filaments which have a much higher bulk than conventional heavy denier yarns containing fewer higher denier filaments.

Whilst the yarns must be stretched to at least 90 percent of their uncrimped lengths, it is preferred that they should be stretched by an amount in excess of this provided that they are not stretched to lengths greater than their uncrimped lengths as this removes some of the crimp in the filaments and can cause filament breakage.

An example of an apparatus for carrying out the process of the invention is shown in the accompanying drawing, in which

FIGURE 1 is a diagrammatic elevation of a stuffing box and

FIGURE 2 is a diagrammatic elevation of a yarn stretching apparatus.

In FIGURE 1, six yarns 1 are drawn from individual yarn packages 2 over a tension device, shown as two tension rolls 3 and are presented to the nip of a pair of feed rollers 4 and 5 through a guide comprising a number of upright comb pins 6 which separate each yarn from its neighbour. The axis of the lower roller 4 is fixed and the upper roller 5 is subjected to downward pneumatic pressure. The yarns are guided by the positioning of the rolls 3 and guide pins 6 so that they are drawn into the nip of rollers 4 and 5 in a single layer, in side-by-side relation, and are fed as a layer into a channel 7 which has electric heaters 8 in its base. The walls of the channel are smooth and the width of the channel is wider than the

sum of the diameters of the yarns, such that the yarns are allowed a degree of lateral movement in the channel. The open top of channel 7 is closed by a pressure plate 9 of T-shape cross-section, the limb of which is of width such as to fit closely but freely between the walls of the channel and of depth somewhat greater than the depth of the channel. Electric heaters 10 are mounted on top of the pressure plate 9 and the plate is pivotally mounted by arms 11 upon the shaft 12 of the upper roller 5. A yoke 13 spans the opposite end of the pressure plate 9 and the adjacent part of the channel 7 enables weights 14 to be applied to it to vary the pressure on the yarn being treated. The yarns emerge from the end of channel 7 in the form of a ribbon 15, adjacent yarns adhering slightly together and each of the yarns being crimped.

In addition to the electric heaters 8 and 10, preparation may be made for steam heating the yarns passing through the crimping channel 7. This is particularly desirable for some yarns where the presence of moisture from the steam is advantageous in setting the crimp. For this purpose a pipe 16 is provided, passing through the base of the channel 7 close to its end adjacent to the rollers 4 and 5 so that steam may be passed into the channel to permeate the yarns at this point.

In FIGURE 2 the ribbon of yarns 15, which may come directly from the stuffing box shown in FIGURE 1 or from storage, is drawn into the nip of a pair of rollers 17 and is then passed to a second pair of rollers 18 which are rotated at a higher surface speed than rollers 17 such that the yarns are stretched between the rollers to at least 90 percent of their uncrimped lengths. Between the pairs of rollers 17 and 18 is a guide comprising a number of comb pins 19 which separate the yarns in the tow 15 so that they emerge as separate yarns 20 from rollers 18 whereupon they are relaxed and collected into packages.

An apparatus as described above, having a crimping channel of approximately 13" long, measured from the axis of rollers 4 and 5 and having an internal width of 0.5" was used in the production of bulked yarns as described in the following examples.

#### Example 1

Three nylon-6 yarns, each of 3000 denier and 4 turns per inch, were fed through the apparatus at a speed of 50 yards per minute with the stuffing box heated to a temperature of 170° C. The crimped yarns withdrawn from the stuffing box as a ribbon were collected in a box and allowed to cool overnight in a conditioned atmosphere. Subsequently, the ribbon was withdrawn from the box, passed over a lick-roller, for the application of an anti-static agent and a lubricant, stretched between two pairs of nip rollers to about 95 percent of the uncrimped length of the yarns and then relaxed and the separate yarns were collected on cones. The yarns were highly bulked and a tufted loop-pile carpet made using the bulked yarns in the pile was found to have excellent properties.

#### Example 2

The procedure of Example 1 was followed with the exception that the three nylon-6 yarns were replaced by thirty 70 denier 0.5 t.p.i. yarns which were fed to the stuffing box as three layers each of 10 yarns. The yarns in the middle and the top layers were superimposed on the appropriate yarns of the bottom layer by using a guide hav-

ing 10 slots, through each of which one yarn from each layer was passed. The speed of the yarns through the stuffing box was increased to 500 yds. per minute.

During the stretching operation the tow or ribbon of 5 yarns was separated into 10 yarns, each formed from three of the original yarns, which were individually collected. A sock knitted from one of these yarns was found to be equivalent in bulk and weight to a sock of similar construction made from 4 ends of a false-twisted yarn of the same type.

#### Example 3

The procedure of Example 2 was followed with the exception that the 30 yarns were replaced by 10 yarns each of 200 denier. The ten yarns formed a single layer.

#### Example 4

The procedure of Example 2 was followed with the exception that the three layers each of 10 yarns were replaced by 18 layers each of three yarns. The product of 20 this example was a heavy denier bulked yarn having a very large number of filaments.

#### Example 5

The procedure of Example 1 was followed except that 25 the yarns used were 1000 denier yarns of an acrylonitrile/vinylidene chloride copolymer.

The products of all the examples had two particular advantages over yarns produced by false-twisting in that the yarns had no twist-bias and had small extensibilities.

30 What I claim is:

1. A yarn bulking process comprising passing a plurality of low-twist, heat-settable, continuous filament yarns, which are parallel to each other and in a single layer, between a pair of nip rollers, into and through a stuffing box 35 of a width such that the yarns are allowed a degree of lateral movement, and having a transverse wall which is defined by a pressure plate which is maintained parallel with the opposite transverse wall, heating the yarns at some stage in their passage into and through the stuffing box, cooling the yarns to set the crimp imposed on them in the stuffing box, stretching the yarns to at least 90 percent of their uncrimped lengths, thereby separating the filaments in the yarns, and then relaxing the yarns, whereupon the filaments tend to revert to the crimped shapes 40 imparted to them in the stuffing box and engagement of adjacent filaments with each other produces a bulking effect on the yarn.

2. A process according to claim 1 wherein a plurality of layers of yarns, each layer comprising a plurality of 45 yarns, are fed to the nip rollers, superimposed yarns being kept close together during the relaxation, whereby the filaments of the adjacent yarns tend to interfere to keep the yarns together.

#### References Cited

##### UNITED STATES PATENTS

|           |        |                    |       |
|-----------|--------|--------------------|-------|
| 3,022,545 | 2/1962 | Wylde et al. ----- | 19—66 |
| 3,044,145 | 7/1962 | Tager -----        | 28—1  |
| 3,099,064 | 7/1963 | Haynes -----       | 28—1  |
| 3,298,079 | 1/1967 | Ageth et al. ----- | 28—72 |
| 3,325,874 | 6/1967 | Edney -----        | 28—1  |
| 3,340,585 | 9/1967 | Buckley et al.     |       |

65 LOUIS K. RIMRODT, Primary Examiner.